

Patented July 21, 1953

2,646,408

# UNITED STATES PATENT OFFICE

2,646,408

## COTTONSEED MEAL GLUES OF LOW ALKALINITY

Jett C. Arthur, Jr., and Joseph T. Hogan, New Orleans, La., assignors to the United States of America as represented by the Secretary of Agriculture

No Drawing. Application May 3, 1951,  
Serial No. 224,439

2 Claims. (Cl. 260—6)

(Granted under Title 35, U. S. Code (1952),  
sec. 266)

1

The invention herein described may be manufactured by or for the Government of the United States of America for governmental purposes throughout the world without the payment to us of any royalty thereon.

This invention relates to the production of glue from cottonseed meal or cake. More particularly it provides glues, which are so produced, which have a pH low enough to bond thin light-colored veneers or pieces of acid woods without discoloring them.

An important and typical application of seed-meal glues is in the manufacture of plywood. The glues used are often derived entirely or in part from seedmeals. The commonly employed glue formula consists of an aqueous suspension of the meal containing up to about 20% (based upon the weight of meal) of one or more of various additives such as CS<sub>2</sub> (usually in conjunction with carbon tetrachloride), lime, silicates, borates, alums and the like which have been found to improve the water resistance and spreadability of the glue. The seedmeal is generally pulverized to a flour-like consistency and suspended or dispersed in a ratio of from about 20 to 40 parts of meal in 100 parts of a sodium hydroxide and lime solution containing the additives and having a pH of at least about 12.

It has been found that glues having this degree of alkalinity (a pH of 12 or more) will stain acid woods and light-colored veneers; and consequently the utilization of cottonseed meal glues has heretofore been limited to the bonding of dark-colored woods and veneers in spite of their advantageously strong and resistant joints and low cost.

Various attempts to produce cottonseed meal glues of low alkalinity have been described. However, such processes often involve mixing pulverized cottonseed meal with compositions such as urea-formaldehyde resins. The urea-formaldehyde resins are glues in their own right. In addition, such resinous glues are several times as expensive as cottonseed meal. The use of the cottonseed meal as an extender for such a resinous glue, produces a glue comparable to those produced by extending the resinous glue with various other fillers such as inedible wheat flour and the like, and the products are much more expensive than the conventional cottonseed meal glues.

We have surprisingly discovered that by dispersing a cottonseed meal in an aqueous solution, containing formaldehyde, in which solution the principal basic ingredient is urea; glues having a pH of less than 8 (less than the pH of the commonly used low alkalinity urea-formaldehyde glues) and a bond shear strength equal to or greater than that of urea-formaldehyde glues, can be produced. The glues so produced

from cottonseed meal have a particular economic advantage since they can consist principally of cottonseed meal, technical grade urea, and technical grade formaldehyde; all of which are low cost materials compared to the urea-formaldehyde resins.

The cottonseed meal glues of low alkalinity provided by the process of this invention can be produced from cottonseed meals or cakes from which the oil was removed by screw-pressing, hydraulic pressing, or by solvent extraction processes or by other de-oiling processes conducted in the conventional manner.

It is well known that the heating of the meals 15 that is sometimes done in conventional pressing operations denatures the protein. Cottonseed meal glues prepared from meal which has not been subjected to extensive heating, form glue joints which are much stronger than those prepared from an extensively heated meal. Glues prepared from solvent extracted meals, in accordance with the process of the invention, constitute a preferred class of compositions provided by the invention. Another preferred class of 20 compositions provided by the invention consists of the glues so produced from cottonseed meals which have been de-oiled in any manner which leaves a meal containing at least 70% soluble nitrogen as determined by suspending 2.5 grams of the meal in 100 ml. of 0.5 M NaCl for 3 hours at 25° C.

A preferred method of producing the glues 25 provided by the invention consists of dispersing the seed meal in an aqueous solution containing urea, allowing the protein to react with the urea, and adding formaldehyde to the mixture.

The process can be conducted at temperatures 30 ranging from 0° to 100° C. but it can be efficiently and economically conducted at substantially 35 room temperature (20 to 40° C.), and the employment of such temperature is, of course, preferred.

The aqueous solution can suitably contain 40 from 0.5 to 3 parts of urea per part of water, but we have found that particularly effective glues 45 are produced by the employment of aqueous solutions containing about 1 to 2 parts by weight of urea per part of water.

The time required for the protein to react 50 with the urea of course varies with the particular cottonseed meal used, the amount of meal used, the extent to which it is pulverized, and the temperature of the reaction. In general, times sufficient for the pulverized cottonseed meal to become completely wetted by the solution are 55 sufficient. When the reaction is conducted at about room temperature using about 0.5 to 1 parts of a cottonseed meal (containing at least 70% soluble nitrogen and passing through a 60 200-mesh screen) per part of water containing

0.5 to 1 part of urea, particularly suitable glues are produced by allowing from about 20 to 40 minutes for the reaction with urea, adding from 0.3 to 0.5 part formaldehyde and 1 to 1.5 parts of water per part of the urea and meal mixture, and maintaining the resultant mixture for from 40 to 80 minutes at 20 to 40° C.

The conventional additives such as carbon disulfide, carbon tetrachloride, silicates, borates, alums, and the like which improve water resistance and/or spreadability can be incorporated in the suspension.

The formaldehyde can be added in any of its conventionally employed forms, but is preferably added in the form of an aqueous solution. The amount of formaldehyde can be varied from 0.5 to 1 part per part of urea. Particularly suitable glues have been produced by adding an amount of formaldehyde about equal to the amount of urea, in the form of an aqueous solution.

The glues provided by the process of this invention can suitably be applied and used in the conventional hot or cold pressing operations.

The viscosity of the glues prepared by the process of the invention will vary depending upon the concentration of meal, urea and formaldehyde and the time they are allowed to stand as well as upon the particular cottonseed meal used. Particularly suitable glues provided by the process of the invention have a viscosity of from 200 to 250 poises.

The pH of the glues provided by the invention will vary principally depending upon the concentration of urea and meal and acidic or basic additives. Preferred glues provided by the process of the invention have a pH of from 7.5 to 7.8, but in general glues provided by the invention having a pH below about 8.5 can be applied to acid or light-colored woods without causing appreciable discoloration.

The following examples are presented to illustrate in greater detail certain modes of practicing the present invention and certain of its characteristics. Since numerous modifications can suitably be employed, the scope of the invention is defined by the claims and is not to be con-

*Effect of urea-formaldehyde solvent for cottonseed meal and processing conditions on the shear strengths of glue joints<sup>1</sup>*

| Glue Composition                | Solids, Percent | Viscosity (1 hour), poises | Spread, lbs./1,000 sq. ft. glue line, dry wt. | pH  | Pressing Conditions         |                            | Shear Strength <sup>2</sup>               |                                           |
|---------------------------------|-----------------|----------------------------|-----------------------------------------------|-----|-----------------------------|----------------------------|-------------------------------------------|-------------------------------------------|
|                                 |                 |                            |                                               |     | Cold, <sup>3</sup> p. s. i. | Hot, <sup>4</sup> p. s. i. | Dry, wood Failure (lbs./sq. in., percent) | Wet, wood Failure (lbs./sq. in., percent) |
| No. 1                           |                 |                            |                                               |     |                             |                            |                                           |                                           |
| 100 grams hexane-extracted meal | 53              | 202                        | 18                                            | 7.5 | 150                         | 150                        | 282-50                                    | 153-30                                    |
| 100 grams urea                  | 53              | 202                        | 18                                            | 7.5 | none                        | 150                        | 284-45                                    | 150-15                                    |
| 100 grams water                 | 53              | 202                        | 18                                            | 7.5 | 150                         | none                       | 153-20                                    | 89-0                                      |
| 270 ml. 37% HCHO                |                 |                            |                                               |     |                             |                            |                                           |                                           |
| No. 2                           |                 |                            |                                               |     |                             |                            |                                           |                                           |
| 50 grams hexane-extracted meal  | 43              | 218                        | 18                                            | 7.8 | 150                         | 150                        | 287-45                                    | 149-10                                    |
| 100 grams urea                  | 43              | 218                        | 18                                            | 7.8 | 200                         | 200                        | 292-45                                    | 159-35                                    |
| 100 grams water                 | 43              | 218                        | 18                                            | 7.8 | 200                         | 200                        | 300-60                                    | 166-30                                    |
| 270 ml. 37% HCHO                |                 |                            |                                               |     |                             |                            |                                           |                                           |
| No. 3                           |                 |                            |                                               |     |                             |                            |                                           |                                           |
| 75 grams hexane-extracted meal  | 44              | 225                        | 14                                            | 7.8 | 200                         | 200                        | 266-20                                    | 140-15                                    |
| 150 grams urea                  |                 |                            |                                               |     |                             |                            |                                           |                                           |
| 100 grams water                 |                 |                            |                                               |     |                             |                            |                                           |                                           |
| 400 ml. 37% HCHO                |                 |                            |                                               |     |                             |                            |                                           |                                           |
| Urea-formaldehyde               | 63              |                            | 19                                            | 8.1 | 200                         | 200                        | 298-45                                    | 163-20                                    |
| Glue, equal parts               | 45              |                            | 19                                            | 8.1 | 200                         | 200                        | 264-20                                    | 127-0                                     |

<sup>1</sup> Meal, urea, and water reacted prior to addition of formaldehyde.

<sup>2</sup> Average of 20 values determined for 3 ply test pieces by tensile shear tester at dry (conditioned at 75° F. and 32% relative humidity for 6 days) and wet (immersed in water for 48 hours at 77° F. prior to testing) conditions.

<sup>3</sup> Cold pressed at 77° F. for 1,440 minutes.

<sup>4</sup> Hot pressed at 237° F. for 5 minutes.

structed as being limited to the details recited in the examples.

#### EXAMPLE 1

5 One hundred parts of oil-free cottonseed meal were mixed with 100 parts of urea and 100 parts of water at 25° C. for ½ hour. Then 270 parts of 37 percent formaldehyde solution were slowly added to the urea-cottonseed meal reaction product. After one hour, the viscosity of the cottonseed meal glue was 202 poises, and the pH of the glue was 7.5.

10 The low alkaline cottonseed meal glue was used to bond wood veneer with minimum alkali staining to yield plywood having dry and wet shear strengths of about 282 and 153 pounds per square inch, respectively.

#### EXAMPLE 2

15 One hundred parts of oil-free cottonseed meal were mixed with 200 parts of urea and 200 parts of water at 25° C. for ½ hour. Then 270 parts of 37 percent formaldehyde solution were slowly added to the urea-cottonseed meal reaction product. After one hour, the viscosity of the cottonseed meal glue was 218 poises, and the pH of the glue was 7.8.

20 The low alkaline cottonseed meal glue was used to bond wood veneer with minimum alkali staining to yield plywood having dry and wet shear strengths of about 300 and 166 pounds per square inch, respectively.

#### EXAMPLE 3

25 One hundred parts of oil-free cottonseed meal were mixed with 200 parts of urea and 133 parts of water at 25° C. for ½ hour. Then 400 parts of 37 percent formaldehyde solution were slowly added to the urea-cottonseed meal reaction product. After one hour, the viscosity of the cottonseed meal glue was 225 poises, and the pH of the glue was 7.8.

30 The low alkaline cottonseed meal glue was used to bond wood veneer with minimum alkali staining to yield plywood having dry and wet shear strengths of about 266 and 140 pounds per square inch, respectively.

#### EXAMPLE 4

Having thus described our invention, we claim:

1. A process for the production of a cottonseed meal glue which comprises: reacting cottonseed meal with urea by suspending an oil-free cottonseed meal in an aqueous solution containing from about 1 to 2 parts urea and from about 1 to 2 parts water per part of meal and maintaining the suspension at from about 20 to 40° C. for from about 20 to 40 minutes; and reacting the reaction product so produced with formaldehyde by mixing it with formaldehyde in the form of an aqueous solution introducing from about 0.3 to 0.5 parts formaldehyde and from about 1 to 1.5 parts water per part of said reaction product and maintaining the resultant 15 mixture at from about 20 to 40° C. for from about

5 40 to 80 minutes until said mixture has a viscosity of from about 200 to 250 poises.

2. The process of claim 1 wherein the cottonseed meal is an oil-free hexane extracted cottonseed meal.

JETT C. ARTHUR, JR.  
JOSEPH T. HOGAN.

## References Cited in the file of this patent

## UNITED STATES PATENTS

| Number    | Name              | Date          |
|-----------|-------------------|---------------|
| 1,245,975 | Satow             | Nov. 16, 1917 |
| 2,249,003 | Julian et al.     | July 15, 1941 |
| 2,332,801 | Leonardson et al. | Oct. 26, 1943 |